# EUROPEAN PATENT SPECIFICATION

(11) **EP 0 587 993 B1**
(45) Date of publication and mention of the grant of the patent: **12.08.1998**
(21) Application number: 93108457.8
(22) Date of filing: 25.05.1993
(51) Int. Cl.: B22F 9/08, B22D 21/00

(54) **High-purity metal melt vessel and the method of manufacturing thereof and purity metal powder producing apparatus**
Gefäss für hochreine Metallschmelze, Verfahren seiner Herstellung sowie Vorrichtung zur Herstellung von hochreinem Metallpulver
Réservoir de métal liquide ultra-pur, son procédé de fabrication ainsi que l'installation de production de poudre métallique très pure

(30) Priority: 25.05.1992 JP 132856/92; 25.05.1992 JP 132857/92
(43) Date of publication of application: 23.03.1994
(73) Proprietor: MITSUBISHI MATERIALS CORPORATION, Chiyoda-ku, Tokyo (JP)
(72) Inventor: Kohmoto, Hiroaki, c/o Chuo-Kenkyusho, Omiya-shi, Saitama-ken (JP); Murahashi, Noriaki, c/o Chuo-Kenkyusho, Omiya-shi, Saitama-ken (JP); Sato, Rokuro, c/o Chuo-Kenkyusho, Omiya-shi, Saitama-ken (JP); Kohno, Tohru, c/o Chuo-Kenkyusho, Omiya-shi, Saitama-ken (JP)
(74) Representative: Müller-Boré & Partner Patentanwälte

(56) References cited:
- EP-A- 0 199 199
- EP-A- 0 420 393
- EP-A- 0 427 379
- US-A- 3 665 083

## Description

### BACKGROUND OF THE INVENTION

### (1) Field of the Invention

The present invention relates to a method of producing a vessel for melting a high-purity metal (referred to simply as "melting vessel") without causing contamination of the metal. The invention also is concerned with an apparatus for melting high-purity metal employing a vessel and with an apparatus for producing powder of high-purity metal with a high degree of uniformity of particle size.

### (2) Description of the Related Art

Hitherto, various methods and techniques including gas-atomizing method have been broadly used in the production of powders, ribbons and foils of high-purity metals. On the other hand, various melting vessels have been proposed for use in these methods and techniques, such as vessels made of tantalum, molybdenum, rhenium or other refractory metal.

The use of such a vessel made of a refractory metal, however, still suffers from a problem in that the metal constituting the vessel is inevitably dissolved into the molten high-purity metal in the vessel so as to contaminate the metal. This problem is serious particularly when the high-purity metal has high melting point and large reactivity.

In order to carry out the gas-atomizing method or a modification of such method, various apparatuses for producing powdered high-purity metal (referred to simply as "powder producing apparatus", hereafter) have been proposed which comprise a melting vessel for melting a high-purity metal therein, and a gas jetting means which directs a gas to the molten high-purity metal falling from the vessel. Improvements also have been achieved in this field of technique, such as the use of a refractory metal, e.g., tantalum, molybdenum or rhenium, as the vessel material. Such improvements, however, are still unsatisfactory for the reason stated above.

The US-A-3665083 discloses an apparatus according to the preamble of claim 1. In particular, there is disclosed an apparatus for melting and recasting a titanium alloy using a refractory crucible. A titanium alloy disc is positioned in the crucible at the discharge outlet, which can be molten in order to discharge the molten metal through the disc to a mold.

The EP-A-199199 discloses a further apparatus for melting a high-purity metal using a melting vessel, in which the lid closing the opening and the bottom of the vessel is made from titanium. The described apparatus uses an arc-generating electrode for melting the metal and the lid.

A problem of the known art is that the known melting vessels do not have any means for adjusting the size of the molten metal outlet port formed in the vessel bottom. Thus, the vessels could not be stably used in the gas atomizing method.

### SUMMARY OF THE INVENTION

Accordingly, it is a primary object of the invention to overcome the above-described problem of the known arts.

It is also an object of the present invention to provide an apparatus which, by employing a vessel, produces powder of a high-purity metal with a high degree of uniformity of the particle size.

It is a further object of the invention to provide a method of producing a melting vessel in a secure and economic way.

The above objects are solved by an apparatus having the features of claim 1 and a method having the features of claim 7 respectively. Preferred embodiments are defined in the respective dependant sub-claims.

According to a preferred embodiment of the present invention, a vessel for melting a high-purity metal comprises a vessel body provided with a cooling jacket and with an opening of a predetermined size formed in the bottom thereof, and a lid made of the same material as the high-purity metal to be molten and closing the bottom opening of the vessel body.

According to another preferred embodiment of the present invention, there is provided an apparatus for melting a high-purity metal, including: a melting vessel having a vessel body provided with an opening of a predetermined size formed in the bottom thereof, and a lid made of the same material as the high-purity metal to be molten and closing the bottom opening of the vessel body; a cooling system for cooling the inner surface region of the vessel body; a beam generating device; a measuring device for measuring the size of an output port formed in the lid and an analyzer; and a control device which controls one or both of the beam output power of the beam generating device and the rate of cooling effected by the cooling system in accordance with the output from the measuring device.

The above and other objects, features and advantages of the present invention will become clear from the following description of the preferred embodiments when the same is read in conjunction with the accompanying drawings.

### BRIEF DESCRIPTION OF THE DRAWINGS

Fig. 1 is a schematic illustration of an embodiment of the melting vessel in accordance with the present invention;
Fig. 2 is a schematic illustration of a method for producing a melting vessel of the type shown in Fig. 1;
Fig. 3 is an illustration of the melting vessel in the state of use;
Fig. 4 is an illustration of an embodiment of a powder producing apparatus in accordance with the present invention; and
Fig. 5 is an illustration of another embodiment of the powder production apparatus.
F ig.6. is an illustration of the particle distribution between the sample of the invention and the conventional sample powder.

### DESCRIPTION OF THE PREFERRED EMBODIMENTS

Briefly, the melting vessel of the present invention has a vessel body having an opening of a predetermined size formed in the bottom thereof, means for cooling the inner surface region of the vessel wall and a lid made of the same material as the metal to be molten in the vessel and closing the bottom opening of the vessel.

The lid may be attached to the vessel body by, for example, preparing the lid of the same metal as the metal to be molten and fitting the lid into the opening. Alternatively, the lid may be formed by a process including the steps of preparing a closure member having a substantially flattened upper surface, closing the bottom opening by the closure member by bringing the latter into abutment with the lower bottom surface of the vessel body, melting a small amount of the metal to be molten in the vessel so as to allow the molten metal to fill the concavity defined by the closure member and the vessel bottom wall surrounding the opening, and allowing the metal to solidify so as to fill the opening.

### Embodiment 1:

Preferred embodiments of the present invention will be described with reference to the drawings.

Referring to Fig. 1 which schematically illustrates an embodiment of the melting vessel of the present invention, the melting vessel has a vessel body denoted by 2 which is a substantially cylindrical cup-like bottom-equipped structure having an internal cavity or recess 8. In this embodiment, the vessel body 2 is made of copper. A tapered opening 10 converging downward is formed in the center of the bottom of the vessel body 2. The vessel body 2 is double-walled to provide a jacket space 12 which communicates with the interior of the pipes 14 and 16 connected to the side wall of the vessel body 2. The arrangement is such that cooling water is supplied into the jacket space 12 through the pipe 14 so as to cool the inner surface region of the vessel body 2 and is then discharged through the pipe 16.

A lid 6 having a tapered outer peripheral surface 6a fits in the opening 10 of the vessel body 2, so as to close the opening 10. This lid 6 is made of the same metal material as the melting object, i.e., the high-purity metal to be molten in the vessel.

Thus, the melting vessel of this embodiment includes the vessel body 2 and the lid 6. The lid 6 may be separately formed in another vessel and then fitted in the opening 10 to close the latter. Alternatively, the lid 6 may be formed by a method which will be described hereinunder with reference to Fig. 2.

### Embodiment 2:

Referring to Fig. 2, there is prepared a closure member 50 having a flattened upper surface. The closure member 50 is brought into abutment with the lower bottom surface of the vessel body 2 to cover the opening 10. Then, a small amount of the metal M, which is the same metal as the high-purity metal to be industrially molten in the vessel 2, is placed in the vessel. This small amount of metal M is then molten by, for example, application of a voltage between the vessel body 2 and the metal M, while the vessel body 2 and the closure member 50 are being cooled. Consequently, the molten metal M flows into the recess 60 defined by the closure member 50 and the bottom wall of the vessel body 2 around the opening 10. The molten metal M is then allowed to solidify within the recess 60. Then, the closure member 50 is removed from the vessel body 2, whereby the lid 6 "fitting" in the opening 10 is obtained in the same form as that shown in Fig. 1.

In operation of the melting vessel of this embodiment, the-melting vessel is charged with an appropriate amount of high-purity metal and is molten by, for example, application of a voltage between the vessel body 2 and the high-purity metal to be molten, while the vessel body is cooled by a cooling medium such as water circulated through the jacket space 12.

Consequently, the portion of the molten high-purity metal contacting the cooled inner wall surface of the vessel body 2 is cooled to solidify so as to form a thin solidified layer or shell covering the entire area of the inner wall surface of the vessel body 2. This solidified metal layer is stably held as long as the cooling of the vessel body 2 is continued. Since the thin solidified metal layer is of the same metal as the high-purity metal molten in the vessel body 2, there is no risk that the metal, i.e., copper constituting the vessel body 2 is molten to contaminate the molten high-purity metal in the vessel body 2.

The lid 6 is not substantially molten because it is cooled as the vessel body 2 is cooled. That is to say, the cooling of the vessel body 2 is so controlled as to satisfy also the demand to maintain the lid 6 in solid state. Upper part of the lid 6 contacting the molten high-purity metal may be molten but this does not cause any contamination of the molten high-purity metal because the lid 6 is of the same high-purity metal as that molten in the vessel body 2.

### Embodiment 3:

The high-purity metal molten in the vessel body 2 is then made to fall downward from the vessel body 2 for the purpose of, for example, production of the metal powder. To this end, as shown in Fig. 3, a beam such as a laser beam, electron beam or a plasma beam is applied to the center of the lid 6 by a beam generator 32 which is disposed right above the lid 6, so that the central portion of the lid 6 is molten by the beam energy so as to form an outlet 6b. The molten high-purity metal is discharged through this outlet 6b. The size of the outlet is easily adjustable by controlling the rate of cooling of the vessel body 2 and the beam power.

As will be understood from the foregoing description, according to the described embodiment of the melting vessel and vessel forming method of the present invention, contamination of the molten high-purity metal, which inevitably occurred in the known art, is avoided whole through the period of operation including the melting period and discharging period in which the molten high-purity metal is discharged downward. In addition, the size of the outlet port for discharging the molten high-purity metal downward can easily be adjusted. Thus, the described embodiments enables steady supply of a molten high-purity metal to a process such as a gas-atomizing powder production process, without any risk of contamination of the molten high-purity metal.

The present invention also provides an apparatus for producing powder of a high-purity metal by using the above-described melting vessel for high-purity metal. According to the invention, in order to attain uniform particle size of the powder, the powder producing apparatus is embodied in various forms as stated below, with specific consideration of the size of the bottom outlet port formed in the lid, as well as the particle size distribution of the powder which is formed by gas-atomization effected on the molten high-purity metal discharged through the bottom outlet port.
(1) An apparatus for producing powder of a high-purity metal, comprising: a melting vessel for melting the high-purity metal therein, the melting vessel including a vessel body having an opening formed in the bottom thereof and a lid which closes the opening and which is made of the same material as the high-purity metal to be molten in the vessel; cooling means for cooling the inner surface region of the vessel body; a gas jetting device which directs a jet of gas towards the downward stream of the molten high-purity metal discharged from the vessel; a beam generating device disposed right above the lid, for applying a beam to the central portion of the lid; a port size detecting means disposed under the lid, for detecting the size of an outlet port formed in the central portion of the lid by the beam; and control means for controlling the rate of cooling effected by the cooling means in accordance with the output from the port size detecting means.
(2) An apparatus for producing powder of a high-purity metal, comprising: a melting vessel for melting the high-purity metal therein, the melting vessel including a vessel body having an opening formed in the bottom thereof and a lid which closes the opening and which is made of the same material as the high-purity metal to be molten in the vessel; cooling means for cooling the inner surface region of the vessel body; a gas jetting device which directs a jet of gas towards the downward stream of the molten high-purity metal discharged from the vessel; a beam generating device disposed right above the lid, for applying a beam to the central portion of the lid; a port size detecting means disposed under the lid, for detecting the size of an outlet port formed in the central portion of the lid by the beam; and control means for controlling the beam output power of the beam generating means in accordance with the output from the port size detecting means.
(3). An apparatus for producing powder of a high-purity metal, comprising: a melting vessel for melting the high-purity metal therein, the melting vessel including a vessel body having an opening formed in the bottom thereof and a lid which closes the opening and which is made of the same material as the high-purity metal to be molten in the vessel; cooling means for cooling the inner surface region of the vessel body; a gas jetting device which directs a jet of gas towards the downward stream of the molten high-purity metal discharged from the vessel; a beam generating device disposed right above the lid, for applying a beam to the central portion of the lid; a port size detecting means disposed under the lid, for detecting the size of an outlet port formed in the central portion of the lid by the beam; and control means for controlling the rate of cooling effected by the cooling means and the beam output power of the beam generating means in accordance with the output from the port size detecting means.
(4) An apparatus for producing powder of a high-purity metal, comprising: a melting vessel for melting the high-purity metal therein, the melting vessel including a vessel body having an opening formed in the bottom thereof and a lid which closes the opening and which is made of the same material as the high-purity metal to be molten in the vessel; cooling means for cooling the inner surface region of the vessel body; a gas jetting device which directs a jet of gas towards the downward stream of the molten high-purity metal discharged from the vessel; a beam generating device disposed right above the lid, for applying a beam to the central portion of the lid; a particle size detecting means disposed under the lid, for detecting the particle size of the high-purity metal powder generated by the jet of gas acting on the downward stream of the molten high-purity metal; and control means for controlling the rate of cooling effected by the cooling means in accordance with the output from the particle size detecting means.
(5) An apparatus for producing powder of a high-purity metal, comprising: a melting vessel for melting the high-purity metal therein, the melting vessel including a vessel body having an opening formed in the bottom thereof and a lid which closes the opening and which is made of the same material as the high-purity metal to be molten in the vessel; cooling means for cooling the inner surface region of the vessel body; a gas jetting device which directs a jet of gas towards the downward stream of the molten high-purity metal discharged from the vessel; a beam generating device disposed right above the lid, for applying a beam to the central portion of the lid; a particle size detecting means disposed under the lid, for detecting the particle size of the high-purity metal powder generated by the jet of gas acting on the downward stream of the molten high-purity metal; and control means for controlling the beam output power of the beam generating means in accordance with the output from the particle size detecting means.
(6) An apparatus for producing powder of a high-purity metal, comprising: a melting vessel for melting the high-purity metal therein, the melting vessel including a vessel body having an opening formed in the bottom thereof and a lid which closes the opening and which is made of the same material as the high-purity metal to be molten in the vessel; cooling means for cooling the inner surface region of the vessel body; a gas jetting device which directs a jet of gas towards the downward stream of the molten high-purity metal discharged from the vessel; a beam generating device disposed right above the lid, for applying a beam to the central portion of the lid; a particle size detecting means disposed under the lid, for detecting the particle size of the high-purity metal powder generated by the jet of gas acting on the downward stream of the molten high-purity metal; and control means for controlling the rate of cooling effected by the cooling means and the beam output power of the beam generating means in accordance with the output from the particle size detecting means.
(7) An apparatus for producing powder of a high-purity metal as stated in one of the foregoing paragraphs (1) to (6), wherein the beam generating device generates one of a laser beam, an electron beam, a plasma beam and an arc beam.

Embodiments of the powder producing apparatus of the present invention will be described hereinunder with reference to the drawings.

Fig. 4 shows an embodiment of the powder production apparatus of the present invention, in which a control is done by adjusting the size or diameter of the outlet port formed in the bottom of the melting vessel. A melting vessel is composed of a vessel body 2 and a lid 6.

The vessel body 2 is a substantially cylindrical cup-shaped bottom equipped vessel having an internal recess 8. A tapered opening 10 is formed in the center of the bottom of the vessel body 2 so as to converge downward. The vessel body 2 is double-walled so that an internal jacket space 12 is formed in communication with pipes 14 and 16 connected to the side wall of the vessel body 2.

The pipe 14 and the pipe 16 are respectively connected to a water supply pipe 22 and a water return pipe 24 of a cooling system 20 which constitutes cooling means. The arrangement is such that cooling water is supplied through the pipe 14 into the jacket space 12 so as to cool the inner surface region of the vessel body 2 and then discharged and collected through the pipe 16. The cooling system 20 supplies cooling water of a constant temperature and has a function to measure the calorific value removed by cooling per unit time (cooling rate) on the basis of the difference between the constant temperature of water supplied into the melting vessel and the temperature of the water collected therefrom, as well as functions to control the initial temperature of the cooling water to be supplied and the volume of the cooling water delivered per unit time.

The lid 6 is made of the same high-purity metal as the high-purity metal which is to be industrially molten in the melting vessel body 2. The lid 6 has a tapered outer peripheral surface 6a which closely fits the tapered wall defining the opening 10 in the vessel body 2 thereby closing the opening 10.

Gas jetting devices 18, 18 disposed under the melting vessel body 2 have nozzles 18a, 18a which jet an inert gas such as Ar gas of a constant pressure to the stream of the molten high-purity metal discharged from the melting vessel body 2, thereby atomizing the molten metal to form particles of the high-purity metal.

A size measurement device 26 such as a camera, disposed near the bottom side of the melting vessel body 2, measures the size, e.g., diameter, of the outlet port formed in the center of the lid 6. The size measuring device 26 is connected to a control device 30 serving as control means, through an analyzer 28 which performs image processing and other operations. The measuring device 26 and the analyzer 28 in cooperation form a port diameter detecting means. The control device 30 includes a central processing unit (CPU), a program ROM and various I/O interfaces.

A beam generating device 32 which is disposed right above the lid 6 emits and directs a beam towards the central portion of the lid 6. The beam generating device 32 is connected to the control device 30 mentioned before. The beam generating device 32 may be of the type which generates a laser beam, an electron beam, a plasma beam or an arc beam.

The control device 30 also is connected to the cooling system 20 to control the cooling rate.

In operation of this embodiment, the melting vessel body 2 is charged with an appropriate amount of high-purity metal and is molten by, for example, application of a voltage between the vessel body 2 and the high-purity metal to be molten, while the inner surface region of the vessel body 2 is cooled by a cooling medium such as water circulated through the jacket space 12.

Consequently, the portion of the molten high-purity metal contacting the cooled inner wall surface 2a of the vessel body 2 is cooled to solidify so as to form a thin solidified layer or shell covering the entire area of the inner wall surface 2a of the vessel body 2. This solidified metal layer is stably held as long as the cooling of the vessel body 2 is continued. Since the thin solidified metal layer is of the same metal as the high-purity metal molten in the vessel body 2, there is no risk that the metal, i.e., copper constituting the vessel body 2 is molten to contaminate the molten high-purity metal in the vessel body 2.

The lid 6 is not substantially molten because it is cooled as the vessel body 2 is cooled. That is to say, the cooling of the vessel body 2 is so controlled as to satisfy also the demand to maintain the lid 6 in solid state. Upper part of the lid 6 contacting the molten high-purity metal may be molten but this does not cause any contamination of the molten high-purity metal because the lid 6 is of the same high-purity metal as that molten in the vessel body 2.

When the melting of the high-purity metal in the melting vessel has reached equilibrium state, a beam is applied by the beam generating device 32 to the central portion of the lid 6 so as to perforate the central region 6b of the lid 6 thereby forming an outlet port. Consequently, the molten high-purity metal inside the vessel body 2 progressively flows out downward through the outlet port, and the downward fall of the molten high-purity metal is cooled and solidified and, in addition, micronized upon collision with the inert gas jetted from the gas jetting devices 18, whereby a powder of the high-purity metal is produced continuously.

Meanwhile, the control device 30 operates to control either one or both of the beam power of the beam generating device 32 and the cooling device 20, based on information concerning the size of the outlet port derived from the measuring device 26 and the analyzer 28, so as to maintain the size of the outlet port constant.

More specifically, the control device 30 operates such that, for example, when the size of the outlet port is greater than an appropriate size, the cooling rate is increased to enhance the effect of cooling of the lid 6 thereby reducing the size of the outlet port, whereas, when the size of the outlet port is smaller than the appropriate value, the beam power is increased relative to the cooling rate so as to apply greater heat to the central region 6b of the lid 6 to enlarge the outlet port.

According to the described embodiment of the powder production apparatus, the size of the outlet port formed in the lid 6 is maintained constant, so that the molten high-purity metal is discharged steadily at a constant rate, thereby ensuring that the produced metal powder has high degree of uniformity of particle size.

### Embodiment 5:

A description will now be given of an embodiment in which a control is done on the basis of the particle size of the high-purity metal powder obtained through gas-atomization, with specific reference to Fig. 5. In this Figure, the same reference numerals are used to denote the same or corresponding parts or portions as those appearing in Fig. 4, and description of such parts or portions is omitted to avoid duplication of explanation.

The powder production apparatus shown in Fig. 5 lacks the size measuring device 26 and the analyzer 28 employed in the embodiment shown in Fig. 4 but, instead, incorporates a particle size measuring device 40 which constitutes particle size detecting means. This particle size measuring device 40 measures particle size of the product powder by making use of laser diffraction. Part of the high-purity metal powder produced through the gas jetting devices 18, 18 is made to pass through the particle size measuring device 40 for measurement of the powder particle size. The output data from the particle size measuring device 40 is delivered to the control device 30.

The process for producing high-purity metal powder in this embodiment is substantially the same as that in the embodiment shown in Fig. 4. In this embodiment, however, the control of the beam output and/or the cooling rate is conducted based upon the powder particle size obtained from the particle size measuring device 40, in contrast to the preceding embodiment of Fig. 4 in which the control is performed in accordance with the data concerning the size of the outlet port derived from the measuring device 26. Thus, the embodiment shown in Fig. 5 ensures that the product powder has a high degree of uniformity of the particle size.

More specifically, the control device 30 operates such that, for example, when the measured powder particle size is greater than an appropriate size, the cooling rate is increased to enhance the effect of cooling of the lid 6 thereby reducing the size of the outlet port, whereas, when the size of the outlet port is smaller than the appropriate value, the beam power is increased relative to the cooling rate so as to apply greater heat to the central region 6b of the lid 6 to enlarge the outlet port.

Thus, in the powder production apparatus of Fig. 5, the flow of the molten high-purity metal discharged from the melting vessel is steadily controlled to ensure that the particle size of the product powder is controlled precisely to a constant size.

Although the invention has been described through its specific forms, it is to be understood that the described embodiments are only illustrative and not intended to limit the scope of the invention.

For instance, the term "high-purity metal" used in this specification should be understood to cover not only pure metals but also alloys and intermetallic compounds.

It is also possible to combine each of the described embodiment with a known technique in which the particle size of the atomized metal is controlled by suitably adjusting the flow rate of the gas jetted from the gas jetting devices.

Other changes and modifications are also possible within the scope of the present invention which is limited solely by the appended claims.

## Claims

1. An apparatus for melting a high-purity metal using a melting vessel comprising a vessel body (2) having an opening (10) of a predetermined size formed in the bottom; and a lid (6) closing said opening (10) and made of the same material as the high-purity metal to be molten in said vessel body (2), **characterized in** that said vessel body (2) has means (12, 20) for cooling inner surface region (8) thereof, and in that the apparatus comprises a beam generating device (32) disposed right above said lid (6), for applying a beam to the central portion of said lid; port size judging means (26; 40), for judging the size of an outlet port (6b) formed in said lid (6) by said beam; control means (28, 30) for controlling the beam output power of said beam generating means (32) and/or the rate of cooling effected by said cooling means (12, 20) in accordance with the output from said port size judging means (26; 40).

2. An apparatus in accordance with claim 1 characterized in that said port judging means (26; 40) comprise port size detecting means (26) disposed under said lid (6), for detecting the size of an outlet port (6b) formed in said lid (6) by said beam.

3. An apparatus in accordance with claim 1 or 2 for producing powder of a high-purity metal, comprising: a gas jetting device (18, 18a) which directs a jet of gas towards the downward stream (34) of the molten high-purity metal discharged from said vessel.

4. An apparatus in accordance with anyone of claims 1 to 3 for producing powder of a high-purity metal, characterized in that said port judging means 26; 40) comprise a particle size detecting means (40) disposed under said lid (6), for detecting the particle size of the high-purity metal powder generated by said jet of gas acting on said downward stream of the molten high-purity metal.

5. An apparatus in accordance with one of the claims 2 to 4, characterized in that said control means (28, 30) control the beam output power of said beam generating means (32) and/or the rate of cooling effected by said cooling means (12, 20) in accordance with the output from said port size detecting means (26) and/or from said particle size detecting means (40).

6. An apparatus according to one of the claims 1 to 5, wherein said beam generating device generates one of a laser beam, an electron beam, a plasma beam and an arc beam.

7. A method of producing a melting vessel, comprising preparing a vessel body (2) having an opening (10) of a predetermined size formed in the bottom and means (12, 20) for cooling inner surface region (8) thereof; forming a lid (6) to close said opening (10) from the same material as the high-purity metal to be molten in said vessel body; and using the steps of closing said opening (10) by bringing a closure member (50) having a substantially flattened upper surface into abutment with the lower bottom surface of said vessel body (2); melting a small amount of said high-purity metal (11) in said vessel body (2) so as to fill the recess (60) formed by said closure member (50) and the bottom wall of said vessel body (2) defining said opening (10) with the molten high-purity metal; allowing the molten high-purity metal to solidify in said recess; and removing said closure member from said vessel body.

8. A method of producing a melting vessel in accordance with claim 7, wherein the steps of preparing a vessel body (2) comprise: cooling inner surface region (8) thereof.

## Patentansprüche

1. Vorrichtung zum Schmelzen eines hochreinen Metalles unter Verwendung eines Schmelzgefäßes, umfassend einen Gefäßkörper (2) mit einer Öffnung (10) einer vorbestimmten Größe, ausgebildet an dem Boden; und einen Deckel (6), die Öffnung (10) verschließend und hergestellt aus demselben Material wie das zu schmelzende hochreine Metall in dem Gefäßkörper (2),
**dadurch gekennzeichnet,** daß
der Gefäßkörper (2) eine Einrichtung (12, 20) aufweist, um den Innenflächenbereich (8) davon zu kühlen, und daß die Vorrichtung umfaßt eine Strahl-Erzeugungseinrichtung (32), angeordnetdirekt über dem Deckel (6), zum Bewirken eines Strahles zu dem Mittelabschnitt des Deckels; eine Portgrößen-Beurteilungseinrichtung (26; 40) zur Beurteilung der Größe des Auslaßports (6b), gebildet an dem Deckel (6) durch den Strahl; eine Steuereinrichtung (28 30) zum Steuern der Strahl-Ausgangsleistung der Strahl-Erzeugungseinrichtung (32) und/oder der Kühlrate, bewirkt durch die Kühleinrichtung (12, 20), und zwar entsprechend der Ausgabe von der Portgrößen-Beurteilungseinrichtung (26; 40).

2. Vorrichtung nach Anspruch 1,
**dadurch gekennzeichnet,** daß
die Port-Beurteilungseinrichtung (26; 40) eine Portgrößen-Erfassungseinrichtung (26) enthält, angeordnet unter dem Deckel (6), zur Erfassung der Größe eines Auslaßports (6b), gebildet an dem Deckel (6) durch den Strahl.

3. Vorrichtung nach Anspruch 1 oder 2 zur Herstellung von Pulver eines hochreinen Metalles, umfassend eine Gas-Strahleinrichtung (18, 18a), welche einen Gasstrahl hin zu der nach unten gerichteten Strömung (34) des geschmolzenen hochreinen Metalles richtet, ausgegeben von dem Gefäß.

4. Vorrichtung gemäß einem der Ansprüche 1 bis 3 zur Herstellung von Pulver eines hochreinen Metalls,
**dadurch gekennzeichnet,** daß
die Port-Beurteilungseinrichtung (26; 40) eine Partikelgrößen-Erfassungseinrichtung (40) umfaßt, angeordnet unter dem Deckel (6), zur Erfassung der Partikelgröße des hochreinen Metallpulvers, erzeugt durch den Gasstrahl, der auf die Nachuntenströmung des geschmolzenen hochreinen Metalls wirkt.

5. Vorrichtung gemäß einem der Ansprüche 2 bis 4,
**dadurch gekennzeichnet,** daß die Steuereinrichtung (28, 30) die Strahl-Ausgangsleistung der Strahl-Erzeugungseinrichtung (32) und/oder die Kühlrate steuert bzw. regelt, bewirkt durch die Kühleinrichtung (12, 20), und zwar entsprechend der Ausgabe von der Portgrößen-Erfassungseinrichtung (26) und/oder von der Partikelgrößen-Erfassungseinrichtung (40).

6. Vorrichtung gemäß einem der Ansprüche 1 bis 5, bei welcher die Strahl-Erzeugungseinrichtung einen Laserstrahl, einen Elektronenstrahl, einen Plasmastrahl oder einen Bogen- bzw. Lichtbogenstrahl erzeugt.

7. Vorrichtung zur Herstellung eines Schmelzgefäßes, umfassend Vorbereiten eines Gefäßkörpers (2) mit einer Öffnung (10) einer vorbestimmten Größe, gebildet an dem Boden, und eine Einrichtung (12 20) zum Kühlen eines Innenflächenbereiches (8) davon; Bilden eines Deckels (6) zum Verschließen der Öffnung (10), aus demselben Material wie das zu schmelzende hochreine Metall in dem Gefäßkörper; und Verwenden der Schritte von Verschließen der Öffnung (10) durch Inanlagebringen eines Verschlußgliedes (50), mit einer im wesentlichen abgeflachten oberen Fläche, mit der unteren Bodenfläche des Gefäßkörpers (2); Schmelzen einer geringen Menge des hochreinen Metalles (11) in dem Gefäßkörper (2), um die Aussparung (60) zu füllen, die durch das Verschlußglied (50) und die Bodenwand des Gefäßkörpers (2) gebildet ist, die Öffnung (10) definierend, mit dem geschmolzenen hochreinen Metall; Ermöglichen, daß das geschmolzene hochreine Metall in der Aussparung sich verfestigt; und Entfernen des Verschlußgliedes von dem Gefäßkörper.

8. Verfahren zur Herstellung eines Schmelzgefäßes nach Anspruch 7, bei welchem die Schritte der Herstellung eines Gefäßkörpers (2) enhalten: Kühlen des Innenflächenbereiches (8) davon.

## Revendications

1. Appareil de fusion d'un métal de grande pureté utilisant un récipient de fusion comprenant un corps formant récipient (2) comportant une ouverture (10) d'une taille prédéterminée formée dans le fond ; et un couvercle (6) fermant ladite ouverture (10) et fait de la même matière que le métal de grande pureté à fondre dans ledit corps formant récipient (2), caractérisé en ce que ledit corps formant récipient (2) possède des moyens (12, 20) pour refroidir la zone de surface intérieure (8) de ce dernier, et en ce que l'appareil comprend un dispositif de production de faisceau (32) disposé juste au-dessus dudit couvercle (6), pour appliquer un faisceau à la partie centrale dudit couvercle ; des moyens de détermination de taille d'orifice (26 ; 40) pour déterminer la taille d'un orifice de sortie (6b) formé dans ledit couvercle (6) par ledit faisceau ; des moyens de commande (28, 30) pour commander la puissance de sortie du faisceau desdits moyens de production de faisceau (32) et/ou la vitesse de refroidissement réalisé par lesdits moyens de refroidissement (12, 20) selon la sortie en provenance desdits moyens de détermination de taille d'orifice (26 ; 40) .

2. Appareil selon la revendication 1, caractérisé en ce que lesdits moyens de détermination d'orifice (26 ; 40) comprennent des moyens de détection de taille d'orifice (26) disposés sous ledit couvercle (6), pour détecter la taille d'un orifice de sortie (6b) formé dans ledit couvercle (6) par ledit faisceau.

3. Appareil selon la revendication 1 ou 2, pour produire une poudre d'un métal de grande pureté, comprenant : un dispositif d'émission de jet de gaz (18, 18a) qui oriente un jet de gaz vers le flot allant vers le bas (34) du métal fondu de grande pureté déchargé dudit récipient.

4. Appareil selon l'une quelconque des revendications 1 à 3, pour produire une poudre d'un métal de grande pureté, caractérisé en ce que lesdits moyens de détermination d'orifice (26 ; 40) comprennent des moyens de détection de taille de particule (40) disposés sous ledit couvercle (6), pour détecter la taille de particule d'une poudre de métal de grande pureté produite par ledit jet de gaz agissant sur ledit flot allant vers le bas du métal fondu de grande pureté.

5. Appareil selon l'une des revendications 2 à 4, caractérisé en ce que lesdits moyens de commande (28, 30) commandent la puissance de sortie du faisceau desdits moyens de production de faisceau (32) et/ou la vitesse de refroidissement réalisé par lesdits moyens de refroidissement (12, 20) selon la sortie en provenance desdits moyens de détection de taille d'orifice (26) et/ou en provenance desdits moyens de détection de taille de particule (40).

6. Appareil selon l'une des revendications 1 à 5, dans lequel ledit dispositif de production de faisceau produit soit un faisceau laser, soit un faisceau d'électrons, soit un faisceau de plasma, et soit un faisceau d'arc.

7. Procédé de production d'un récipient de fusion, comprenant la préparation d'un corps formant récipient (2) comportant une ouverture (10) d'une taille prédéterminée formée dans le fond et des moyens (12, 20) pour refroidir la zone de surface intérieure (8) de ce dernier ; la préparation d'un couvercle (6) pour fermer ladite ouverture (10) à partir de la même matière que le métal de grande pureté à fondre dans ledit corps formant récipient ; et l'utilisation des étapes de fermeture de ladite ouverture (10) en amenant un élément de fermeture (50), ayant une surface supérieure sensiblement aplatie, en butée contre la surface de fond inférieure dudit corps formant récipient (2) ; la fusion d'une petite quantité dudit métal de grande pureté (11) dans ledit corps formant récipient (2) de façon à remplir l'évidement (60) formé par ledit élément de fermeture (50) et la paroi de fond dudit corps formant récipient (2) définissant ladite ouverture (10) avec le métal fondu de grande pureté ; l'autorisation de solidification du métal fondu de grande pureté dans ledit évidement ; et de retrait dudit élément de fermeture dudit corps formant récipient.

8. Procédé de production d'un récipient de fusion selon la revendication 7, dans lequel les étapes de préparation d'un corps formant récipient (2) comprennent : le refroidissement de la zone de surface intérieure (8) de ce dernier.
